

## UNITED STATES PATENT OFFICE

LLOYD C. SWALLEN AND WILLIAM J. BANNISTER, OF TERRE HAUTE, INDIANA, AS  
SIGNORS TO COMMERCIAL SOLVENTS CORPORATION, OF TERRE HAUTE, INDIANA,  
A CORPORATION OF MARYLAND

## CHEMICAL COMPOUND AND METHOD OF MAKING THE SAME

No Drawing.

Application filed March 18, 1928. Serial No. 262,985.

Our invention relates to the production of a new type of complex chemical compounds which may best be described as metal salts of alkyl acid esters of polybasic acid esters of polyhydric alcohols and polybasic acids. Zinc butyl glyceryl phthalate may be cited as an example of this type of compound. These compounds are valuable as plasticizing substances for cellulose esters, as components of synthetic resins, and for other purposes.

The types of compounds contemplated, the method of reaction, and the structures produced are best illustrated by the following type equations in which

15



represent polyhydric alcohols, R'-OH a

20



The next step involves the preparation of the half ester of the above compounds by reacting them with appropriate quantities of monohydric alcohols. Usually, this operation is carried out as a separate step but in some cases it may be desired to combine the two steps into one operation.

25



30

monohydric alcohol, A(COOH)<sub>2</sub>, a polybasic acid, and MX a metal salt.

35 In preparing a compound of the character in which we are interested, a polyhydric alcohol is first allowed to react with a polybasic acid or anhydride. The product formed depends upon the character of the materials used as well as the method of conducting the reaction. As for example, the reaction may be conducted so as to give compounds having one or more free hydroxyl groups in the polyhydric component. The following equations illustrate the different types of compounds which may be obtained in this step of our process, the reactions being shown as taking place with both dihydric and trihydric alcohols.

We have found that the most convenient method of obtaining the metal salts of the half esters of the type illustrated above is to first prepare the sodium salt and then react this compound with a salt of the metal which it is desired to substitute for the sodium radical. For example,



If the metal, the salt of which is to be formed, is divalent, the compound formed during the next reaction may be represented as follows:





- 5 In case a trihydric alcohol has been used as the starting material and all of its hydroxyl groups have been neutralized, as shown under Equation III above, a compound of the following character will be obtained with a divalent metal:



- 15 When a dihydric alcohol is used in place of a trihydric, the final product similarly becomes of the character indicated by the formula:



- We shall now describe the preparation of a number of specific examples.

### EXAMPLE 1

25 *Sodium butyl glyceryl phthalate*

138 grams of anhydrous glycerol and 444 grams of phthalic anhydride were heated together for about one hour at approximately 30 150° C. After cooling somewhat, 400 grams of butyl alcohol, 15 grams of concentrated sulphuric acid (catalyst) and about 400 c. c. of benzol were added to the reaction mixture and the heating continued. The water 35 formed during the reaction was removed by distillation, as a component of a constant boiling mixture, with the benzol. Fresh additions of the benzol were made to the reaction mixture from time to time so as to maintain 40 the reaction temperature between 90° and 100° C. This was continued until 27 c. c. of water had separated (half the amount required for complete esterification). The product thus formed was poured into water, 45 and neutralized with 550 c. c. of 2.75 N NaOH, which gave sodium butyl glyceryl phthalate, together with a small amount of glyceryl butyl phthalate and some unused butyl alcohol. The butyl alcohol was removed by distillation in vacuo, the residue diluted to 50 about six liters and finally extracted two or three times with benzol to remove the glyceryl butyl phthalate.

### EXAMPLE II

55 *Zinc butyl glyceryl phthalate*

The first step involved the preparation of sodium butyl glyceryl phthalate, which was obtained as described above under Example I.

60 Upon the addition of a solution, containing an amount of zinc chloride in excess of that theoretically required, say 240 grams, to the sodium butyl glyceryl phthalate, a precipitation of the zinc butyl glyceryl phthalate immediately took place. After washing

65

the zinc salt with distilled water, the latter was separated as completely as possible, and the salt dissolved in butyl alcohol. The solution was filtered and the water and butyl alcohol then removed by distillation in vacuo, until the temperature of the liquid rose to 130° C. 70

Zinc butyl glycerl phthalate, obtained in this manner, is a liquid of the consistency of soft taffy. Its color is light straw to colorless, depending upon the purity. It is soluble in butyl alcohol, butyl acetate, dibutyl phthalate, ethyl alcohol and benzol. It is insoluble in water and "V. M. P. naphtha". 75

### EXAMPLE III

### *Calcium butyl glyceryl phthalate*

Sodium butyl glyceryl phthalate obtained as described under Example I, was treated with a solution, containing an amount of anhydrous calcium chloride in excess of that theoretically required, say 150 grams. The product obtained was washed with water, dissolved in butyl alcohol, filtered, and the water and butyl alcohol finally removed by distillation in vacuo, as described under Example II.

The calcium butyl glyceryl phthalate obtained by this method closely resembled the zinc salt described under Example II above, in all the properties studied. 95

#### EXAMPLE IV

### *Copper butyl glyceryl phthalate*

Sodium butyl glyceryl phthalate obtained 100  
as described under Example I, was treated  
with a solution containing an amount of  
crystalline copper nitrate in excess of that  
theoretically required, say 300 grams. The  
precipitate formed was treated as described 105  
under previous examples.

Copper butyl glyceryl phthalate is a clear, dark, green-blue liquid of the consistency of hard taffy. It is soluble in butyl alcohol, butyl acetate, dibutyl phthalate, ethyl alcohol and benzol. It is insoluble in water and "V. M. P. naphtha".

### EXAMPLE V

### *Zinc isoamyl glyceryl phthalate*

Sodium isoamyl glyceryl phthalate was first prepared by reacting 46 grams of anhydrous glycerol, 148 grams of phthalic anhydride and 100 grams of isoamyl alcohol in the presence of 5 grams of concentrated sulphuric acid (catalyst) and benzol, the operation being carried out in two separate steps, as described above under Example I. 120

The zinc isoamyl glyceryl phthalate was then obtained by adding to the sodium isoamyl glyceryl phthalate a solution containing an amount of zinc chloride in excess of that theoretically required, say 80 grams, and treating the resulting compound as described under Example II. 130

Zinc isoamyl glyceryl phthalate resembles closely the corresponding butyl compound in appearance and properties, except for the fact that it is much less viscous than the butyl compound.

5 In the examples described above, we have chosen to use phthalic acid (anhydride) due to its stability, cheapness, and ease of reaction. We may, however, employ other polybasic acids such as terephthalic acid, tar-

10 taric acid, citric acid or the like.

15 Of the various polyhydric alcohols, glycerol and ethylene glycol are best suited for use. Any monohydric alcohol may be used, but we prefer to employ normal butyl alcohol.

20 In place of the sulphuric acid used as a catalyst in the specific examples above disclosed, other esterification catalysts such as hydrochloric acid or phosphoric acid may be used. In place of benzol, other inert liquids forming constant-boiling mixtures with water, for example—carbon tetrachloride—may be employed.

25 Now having described our invention, we claim the following as new and novel:

30 1. A compound having the following structural formula, in which R is a polyhydric alcohol having one hydroxyl group which is unchanged; R' is a monohydric alcohol group; A is a polybasic acid group; and M is a metal:



35 2. A compound having the following structural formula, in which R is a polyhydric alcohol having one hydroxyl group which is unchanged; R' is a monohydric alcohol group; A is a polybasic acid group; and M is a metal:



40 3. A compound as described in claim 2, in which said polyhydric alcohol is glycerine, and said polybasic acid is phthalic acid, said product having the following structural formula:



45 4. A compound as described in claim 2, in which said polyhydric alcohol is glycerine, said polybasic acid is phthalic acid, and said monohydric group is the butyl group.

50 5. A compound as described in claim 2, in which said polyhydric alcohol is glycerine, said polybasic acid is phthalic acid, said monohydric group is the butyl group and the metal is zinc.

55 6. As a new compound, a metal salt of the

alkyl acid ester of the polybasic acid ester of a polyhydric alcohol and a polybasic acid.

7. As a new compound, a polyvalent metal salt of the alkyl acid ester of the polybasic acid ester of a polyhydric alcohol and a poly-

70

8. As a new compound, the zinc salt of the alkyl acid ester of the polybasic acid ester of a polyhydric alcohol and a polyvalent acid.

75

9. As a new compound, a metal salt of the butyl acid ester of the polyvalent acid ester of a polyhydric alcohol and a polybasic acid.

10. As a new compound, a polyvalent metal salt of the butyl acid ester of the polyvalent acid ester of a polyhydric alcohol and a polybasic acid.

80

11. As a new compound, a metal salt of the alkyl acid ester of the monophthalate ester of a polyhydric alcohol.

90

12. As a new compound, a polyvalent metal salt of the butyl acid ester of the monophthalate ester of a polyhydric alcohol.

13. As a new compound, a metal salt of the butyl acid ester of the monophthalate ester of glycerol.

95

14. As a new compound, a polyvalent metal salt of the butyl acid ester of the monophthalate ester of glycerol.

15. The process of manufacturing the metal salt of an alkyl acid ester of the polybasic acid ester of a polyhydric alcohol and a polybasic acid which comprises reacting a polybasic acid or anhydride with a polyhydric alcohol; adding a monohydric alcohol, a catalyst, and benzol to the reaction mixture; removing water from the reaction mixture as a component of a constant-boiling mixture until the reaction has proceeded to the desired extent; washing and neutralizing with an alkaline hydroxide, the product thus obtained; and finally reacting said neutralized product with a metal salt and recovering the material thus formed.

100

105

16. In testimony whereof we affix our signatures.

LLOYD C. SWALLEN.  
WILLIAM J. BANNISTER.

110

115

120

125

130